# EUROPEAN PATENT APPLICATION

(11) **EP 2 565 257 A1**
(43) Date of publication of application: **06.03.2013**
(21) Application number: 10850795.5
(22) Date of filing: 27.05.2010
(51) Int. Cl.: C10M 169/04, C10M 101/02, C10M 129/72

(54) **FIRE-RESISTANT HYDRAULIC OIL**

(30) Priority: 27.04.2010 KR 20100038955
(71) Applicant: Hannal Inc., Ulju-gun, Ulsan 336-893 (KR)
(72) Inventor: KIM, Kwang Soon, Seoul 135-110 (KR); KIM, Doo Myung, Seoul 135-090 (KR); BAIK, Sun Ki, Cheonan-si, Chungcheongnam-do 331-734 (KR); LEE, Dong Choon, Asan-si, Chungcheongnam-do 336-712 (KR)
(74) Representative: Witte, Weller & Partner
(86) International application number: PCT/KR2010/003368
(87) International publication number: WO 2011/136429

(57) **Abstract**

Provided is a flame-retardant hydraulic oil prepared by mixing 25 to 97 % by weight (wt%) of a petroleum lubricating base oil, 1 to 20 wt% of a phosphorus or halogen flame-retardant additive, 1 to 35 wt% of an ester compound, and 0.05 to 20 wt% of a performance enhancer.

## Description

### Technical Field

The present invention relates to a new type of flame-retardant hydraulic oil which is impervious to fire and has heat and oxidation stability to lengthen a life, contributing to social development and stability.

### Background Art

As an increasing number of high-temperature and high-pressure devices are being used in a variety of industrial facilities, it is necessary to supply a lubricating oil, in particular, hydraulic oil which may actively contribute to addressing a risk of fire. A hydraulic oil which contributes to dealing with a risk of fire is referred to as a flame-retardant hydraulic oil and is classified as follows in Table 1, according to the International Organization for Standardization (ISO) standards ISO classification system.

A flame-retardant hydraulic oil collectively refers to products which cause small flames, does not allow a fire to quickly spread, and is self-extinguishable when a fire breaks out.

Various types of hydraulic oils are currently being developed and used, wherein petroleum hydraulic oils including mineral oils as lubricating base oils are mostly used. However, the petroleum, that is, mineral hydraulic oils are inappropriate for use at high-temperatures due to a great risk of fire. In contrast, the flame-retardant hydraulic oil is safe from a fire and is very expensive, for example, 3 to 10 times a price of petroleum oils and needs to be handled in a special environment, for example, for sealing and packing. Thus, many facilities use petroleum hydraulic oils in a dangerous environment in which exposure to a fire is prevalent.

Therefore, a need exists for a new, inexpensive type of flame-retardant hydraulic oil that does not need to be handled in a special environment, and is usable for a long period of time.

### Disclosure of Invention

### Technical Goals

An aspect of the present invention provides a flame-retardant hydraulic oil which is fire resistant, inexpensive, does not need to be handled in a special environment, and has a long life.

### Technical solutions

According to an aspect of the present invention, there is provided a flame-retardant hydraulic oil prepared by mixing 25 to 97 % by weight (wt%) of a petroleum lubricating base oil, 1 to 20 wt% of a phosphorus or halogen flame-retardant additive, 1 to 35 wt% of an ester compound, and 0.05 to 20 wt% of a performance enhancer.

The petroleum lubricating base oil may include most refined petroleum lubricating base oils provided domestically and internationally, wherein a petroleum lubricating base oil having a dynamic viscosity of 5 to 1,000 millimeters/second (mm²/sec) at 40 °C and a paraffin content of 50 to 90 wt% is preferably used since petroleum lubricating base oils having excessively high or excessively low viscosity may cause a problem in operation.

The flame-retardant additive used for the flame-retardant hydraulic oil may include phosphorus or halogen flame-retardant additives, wherein a compound including both phosphorus and halogen additives further enhances flame retardancy. The flame-retardant additive is obtained by introducing phosphorus and a halogen, which are flame retardant, into an aryl or allyl group and is selected from the group consisting of tricresyl phosphate, tributyl phosphate, tris(β-chloroethyl) phosphate, tris(β-chloropropyl) phosphate, tris(dichloropropyl) phosphate, trioctyl phosphate, triphenyl phosphate, octyl diphenyl phosphate, tris(isopropylphenyl) phosphate and tributoxyethyl phosphate.

The ester compound used for the flame-retardant hydraulic oil may include at least one selected from the group consisting of compounds represented by Formulas 1 to 3: where R₁ and R₂ are the same or different and each represent a C1 to C2 alkyl group, and R₃ and R₄ are the same or different and each represent a C6 to C22 saturated or unsaturated alkyl group; where R₁ represents a C1 to C2 alkyl group, and R₂, R₃ and R₄ are the same or different and each represent a C6 to C22 saturated or unsaturated alkyl group; and where n is an integer from 2 to 12, and R₁ and R₂ are the same or different and each represent a C2 to C 18 alkyl group.

The ester compound may include polyol esters disclosed by the inventor of the present invention in KR Patent Registration No. 88842, No. 169565 and No. 0201759 and may include at least one of dibasic esters, such as adipates, azelates, sebacates and phthalates.

The hydraulic oil is inexpensive, does not need to be handled in a special environment and has excellent flame retardancy by adding the phosphorus or halogen flame-retardant additive to the petroleum lubricating base oil. Conventionally, the phosphorus or halogen flame-retardant additive is not properly mixed into the petroleum lubricating base oil, but the present invention solves such a problem by adding the ester compound.

According to an aspect of the present invention, the performance enhancer includes an antioxidant, an anti-load and anti-abrasive additive, a viscosity enhancer, an anticorrosive agent and an antifoaming agent.

The antioxidant may include metal salts of phenylnaphthylamine, phenyl, and phosphate ester and be used in an amount of 0.1 to 10 wt%.

The anti-load and anti-abrasive additive is preferably amine salts of phosphate ester neutralized and represented by Formula 4, has a synergy effect in combination with metal salts of phosphate ester, allyl phosphate ester and a sulfide as additives, and is added in an amount of 0.05 to 7.0 wt%: where R represents hydrogen or a C1 to C10 alkyl or aryl hydrocarbon compound, X represents hydrogen or C1 to C4 hydrocarbon, and n is an integer from 1 to 10.

The viscosity enhancer may include an olefin copolymer, polymethacrylate or the like, preferably polymethacrylate exhibiting excellent shear stability and less change in viscosity and having a molecular weight of 200,000 or less. Here, a combination of a low molecular weight viscosity enhancer and a high molecular weight viscosity enhancer may improve low-temperature fluidity as well as viscosity index. The viscosity enhancer is added in an amount of 0.1 to 5.0 wt%.

0.01 to 2.0 wt% of the anticorrosive agent or the antifoaming agent may be added, as necessary.

Although the foregoing additives are necessary for the lubricating oil composition, excessive amounts thereof may reduce flame retardancy or decrease in viscosity by shear, generation of dregs or discoloration of the oiling agent. Thus, it is needed to mix proper amounts of the base oil and the additives.

### Advantageous effects

A flame-retardant hydraulic oil according to the present invention is safe from a fire, inexpensive, does not need to be handled in a special environment, and has a long life.

### Brief Description of Drawings

FIG. 1 is a diagram illustrating occurrences of sludge in examples of the present invention and comparative examples after an oxidation stability test.

### Best Mode for Carrying Out the Invention

Reference will now be made in detail to embodiments of the present invention.

### Preparation of petroleum (mineral) lubricating base oil

As a petroleum lubricating base oil, general lubricating base oils available from oil companies were used in view of a flash point, heat and oxidation stability, and impurities content as illustrated in Table 2.

**Table 2**

| | Dynamic viscosity (mm²/sec) | Color (KS M 2106) | Flash point (in open cup, °C) | Hydrocarbon composition | |
|---|---|---|---|---|---|
| | | | | Cₚ | C_{A} |
| Petroleum lubricating base oil A | 15.0 ± 2.0 | 2.5 or lower | 200 or higher | 50 or higher | 3 or lower |
| Petroleum lubricating base oil B | 20.0 ± 2.0 | | 200 or higher | | |
| Petroleum lubricating base oil C | 30.0 ± 2.0 | | 220 or higher | | |
| Petroleum lubricating base oil D | 35.0 ± 2.0 | | 220 or higher | | |
| Petroleum lubricating base oil F | 50.0 ± 2.0 | | 240 or higher | | |
| Petroleum lubricating base oil H | 100.0 ± 5.0 | | 240 or higher | | |
| Petroleum lubricating base oil G | 120.0 ± 10.0 | | 260 or higher | | |
| Petroleum lubricating base oil H | 200.0 ± 10.0 | | 260 or higher | | |
| Petroleum lubricating base oil I | 480.0 ± 20.0 | | 300 or higher | | |
| Petroleum lubricating base oil J | 1000.0 ± 100.0 | | 300 or higher | | |
| The closer to 0.0 C_{A} is, the more appropriate. | | | | | |

### Preparation of ester lubricating base oil

Ester compounds used to prepare mixed flame-retardant hydraulic oils according to the present invention were prepared as listed in Table 3 and may be used independently or as mixtures.

**Table 3**

| | Type I (self-manufactured ester) | Type II (commercially available ester) |
|---|---|---|
| Appearance (KS M 2106) | 2.5 or lower | 2.5 or lower |
| Total acid number (mg KOH/g) | 3.0 or lower | 2.0 or lower |
| Dynamic viscosity (40°C), mm²/sec) | 20 to 120 | 10 to 250 |
| Flash point (open type, °C) | 250 or higher | 200 or higher |

### Preparation of flame-retardant additive

Flame-retardant additives were prepared as illustrated in Table 4, wherein raw materials having a purity of 80% or higher were used for stability of the hydraulic oils.

**Table 4**

| | |
|---|---|
| Flame-retardant additive A | Tricresyl phosphate |
| Flame-retardant additive B | Tributyl phosphate |
| Flame-retardant additive C | Tris(β-chloroethyl) phosphate |
| Flame-retardant additive D | Tris(β-chloropropyl) phosphate |
| Flame-retardant additive E | Tris(dichloropropyl) phosphate |
| Flame-retardant additive F | Trioctyl phosphate |
| Flame-retardant additive G | Triphenyl phosphate |
| Flame-retardant additive H | Octyl diphenyl phosphate |
| Flame-retardant additive I | Tris(isopropylphenyl)phosphate) |
| Flame-retardant additive J | Tributoxyethyl phosphate |

### Preparation of hydraulic oil

The lubricating base oils and the flame-retardant additives listed in Tables 2, 3 and 4 were added to suitable amounts of performance enhancers, thereby preparing hydraulic oils as illustrated in Tables 5 and 6. Here, content is expressed as percent by weight (wt%).

**Table 5**

| Ingredients | Example 1 | Example 2 | Example 3 | Example 4 | Example 5 | Example 6 | Example 7 |
|---|---|---|---|---|---|---|---|
| Petroleum lubricating base oil A | 20.0 | | 40.0 | | | | |
| Petroleum lubricating base oil C | | 65.0 | | 30.0 | | | |
| Petroleum lubricating base oil E | 60.0 | 20.0 | | 40.0 | 70.0 | | |
| Petroleum lubricating base oil G | | | 40.0 | | | 40.0 | 10.0 |
| Petroleum lubricating base oil I | | | | | 10.0 | 25.0 | 40.0 |
| Self-manufactured ester 1 | 5.0 | | 10.0 | | | 10.0 | |
| Commercially available ester 2 | | 3.0 | | 5.0 | | | 30.0 |
| Flame-retardant additive A | 2.0 | | 2.0 | | 5.0 | | |
| Flame-retardant additive B | 5.0 | 3.0 | | | | | |
| Flame-retardant additive C | | | 1.0 | | | | |
| Flame-retardant additive D | | | | 10.0 | | | |
| Flame-retardant additive E | | 3.0 | | | | | |
| Flame-retardant additive F | | | | | | 10.0 | |
| Flame-retardant additive G | | | | | | 10.0 | |
| Flame-retardant additive H | | | 2.0 | 5.0 | | | |
| Flame-retardant additive I | | | | | 5.0 | | |
| Flame-retardant additive J | | | | | | | 10.0 |
| Antioxidant | 1.0 | 0.5 | 2.0 | 1.0 | 0.5 | 2.0 | 0.5 |
| Anti-abrasive additive | 1.0 | 0.5 | 2.0 | 2.0 | 2.0 | 2.0 | |
| Viscosity enhancer | Suitable | Suitable | Suitable | Suitable | Suitable | Suitable | Suitable |
| Antifoaming agent and etc. | Suitable | Suitable | Suitable | Suitable | Suitable | Suitable | Suitable |

**Table 6**

| Ingredients | Example 8 | Example 9 | Example 10 | Example 11 | Example 12 | Example 13 | Example 14 |
|---|---|---|---|---|---|---|---|
| Petroleum lubricating base oil B | 60.0 | | 20.0 | | | | |
| Petroleum lubricating base oil D | | 50.0 | | 30.0 | | | |
| Petroleum lubricating base oil F | | 20.0 | | 20.0 | 45.0 | | |
| Petroleum lubricating base oil H | 10.0 | | 50.0 | | | 40.0 | |
| Petroleum lubricating base oil J | | | | | | | 15.0 |
| Self-manufactured ester 1 | 10.0 | | 10.0 | | 35.0 | 35.0 | |
| Commercially available ester 2 | | 5.0 | | 20.0 | | | 20.0 |
| Flame-retardant additive A | 5.0 | | | 15.0 | 5.0 | | 15.0 |
| Flame-retardant additive B | | 5.0 | | | | | |
| Flame-retardant additive C | | | 10.0 | | | | 5.0 |
| Flame-retardant additive D | 5.0 | | | | 10.0 | | |
| Flame-retardant additive E | | 5.0 | | | | | |
| Flame-retardant additive F | | | | 5.0 | | | |
| Flame-retardant additive G | 5.0 | | | | | 20.0 | |
| Flame-retardant additive H | | | 10.0 | | | | |
| Flame-retardant additive I | | 5.0 | | | | | |
| Flame-retardant additive J | | | 5.0 | | | | |
| Antioxidant | 1.0 | 1.0 | 2.0 | 1.0 | 1.5 | 1.0 | 0.5 |
| Anti-abrasive additive | 2.0 | 1.0 | 2.0 | 2.0 | 2.0 | | 1.0 |
| Viscosity enhancer | Suitable | Suitable | Suitable | Suitable | Suitable | Suitable | Suitable |
| Antifoaming agent and etc. | Suitable | Suitable | Suitable | Suitable | Suitable | Suitable | Suitable |

### Quality test of flame-retardant hydraulic oils

The hydraulic oils prepared as illustrated in Tables 5 and 6 were evaluated in terms of qualities, and results thereof are listed in Tables 7 and 8.

The hydraulic oils were generalized in accordance with the International Standards Organization Viscosity Grade (ISO VG). Oxidation stability was evaluated by the rotating bomb oxidation test, ASTM D 2272, while abrasion resistance was evaluated by the shell 4-ball test. Further, flame retardancy was evaluated by the hot manifold test, MIL-F-7100 Fed 6053, in which a sample was dropped on a manifold at a temperature of 374 °C and identified whether to ignite, and by a sprayed fire test, by which a sample is accessed as flame retardant when the sample has an oxygen demand of 50% or higher necessary to catch fire when sprayed.

**Table 7**

| Ingredients | Example 1 | Example 2 | Example 3 | Example 4 | Example 5 | Example 6 | Example 7 |
|---|---|---|---|---|---|---|---|
| Dynamic viscosity (ISO VG) | 32 | 32 | 46 | 46 | 68 | 68 | 100 |
| Flash point (°C) | 250 | 250 | 250 | 260 | 270 | 270 | 300 |
| Pour point (°C) | -30.0 | -30.0 | -25.0 | -25.0 | -25.0 | -25.0 | -20.0 |
| Oxidation stability (RBOT, min) | 500 | 400 | 400 | 500 | 350 | 400 | 500 |
| Abrasion resistance (Scar ϕ mm) | 0.35 | 0.35 | 0.35 | 0.30 | 0.30 | 0.35 | 0.35 |
| Flame retardancy | Hot Manifold test | Extinguished immediately after ignition | | | | | |
| | Sprayed fire test | Oxygen demand: 50 - 55 % | | | | | |

**Table 8**

| Test categories | Example 8 | Example 9 | Example 10 | Example 11 | Example 12 | Example 13 | Example 14 |
|---|---|---|---|---|---|---|---|
| Dynamic viscosity (ISO VG) | 46 | 46 | 68 | 68 | 68 | 100 | 100 |
| Flash point (°C) | 250 | 260 | 250 | 270 | 270 | 280 | 280 |
| Pour point (°C) | -25.0 | -25.0 | -25.0 | -25.0 | -25.0 | -20.0 | -20.0 |
| Oxidation stability (RBOT, min) | 400 | 400 | 400 | 500 | 600 | 500 | 500 |
| Abrasion resistance (Scar ϕ mm) | 0.30 | 0.35 | 0.35 | 0.35 | 0.35 | 0.35 | 0.30 |
| Flame retardancy | Hot Manifold test | Extinguished immediately after ignition | | | | | |
| | Sprayed fire test | Oxygen demand: 50 ∼ 55 % | | | | | |

### Identification of excellent heat and oxidation stability

When a hydraulic oil is subjected to the rotating bomb oxidation test, discoloration and a large amount of precipitate generally occur, and such a precipitate is identified to cause various faults when equipment operates.

FIG. 1 is a diagram illustrating occurrences of sludge in examples of the present invention and comparative examples after an oxidation stability test.

Referring to FIG. 1, the flame-retardant hydraulic oils according to the examples of the present invention involve less discoloration and generate a small amount of sludge after being tested over a long period of time when compared to a petroleum hydraulic oil and a synthetic hydraulic oil.

Although a few embodiments of the present invention have been shown and described, the present invention is not limited to the described embodiments. Instead, it would be appreciated by those skilled in the art that changes may be made to these embodiments without departing from the principles and spirit of the invention, the scope of which is defined by the claims and their equivalents.

## Claims

1. A flame-retardant hydraulic oil prepared by mixing 25 to 97 % by weight (wt%) of a petroleum lubricating base oil; 1 to 20 wt% of a phosphorus or halogen flame-retardant additive, 1 to 35 wt% of an ester compound, and 0.05 to 20 wt% of at least one performance enhancer selected from the group consisting of an antioxidant, an anti-load and anti-abrasive additive, a viscosity enhancer, an anticorrosive agent and an antifoaming agent.

2. The flame-retardant hydraulic oil of claim 1, wherein the petroleum lubricating base oil has a dynamic viscosity of 5 to 1000 millimeters squared/second (mm²/sec) at 40 °C and has a paraffin content of 50 to 90 wt%.

3. The flame-retardant hydraulic oil of claim 1, wherein the phosphorus or halogen flame-retardant additive comprises a phosphorus and halogen-introduced aryl or allyl group.

4. The flame-retardant hydraulic oil of claim 1, wherein the phosphorus or halogen flame-retardant additive comprises at least one selected from the group consisting of tricresyl phosphate, tributyl phosphate, tris(β-chloroethyl) phosphate, tris(β-chloropropyl) phosphate, tris(dichloropropyl) phosphate, trioctyl phosphate, triphenyl phosphate, octyl diphenyl phosphate, tris(isopropylphenyl) phosphate and tributoxyethyl phosphate.

5. The flame-retardant hydraulic oil of claim 1, wherein the ester compound comprises at least one selected from the group consisting of compounds represented by Formulas 1 to 3: where R₁ and R₂ are the same or different and each represent a C1 to C2 alkyl group, and R₃ and R₄ are the same or different and each represent a C6 to C22 saturated or unsaturated alkyl group; where R₁ represents a C1 to C2 alkyl group, and R₂, R₃ and R₄ are the same or different and each represent a C6 to C22 saturated or unsaturated alkyl group; and where n is an integer from 2 to 12, and R₁ and R₂ are the same or different and each represent a C2 to C18 alkyl group.

6. The flame-retardant hydraulic oil of claim 1, wherein the ester compound comprises at least one selected from the group consisting of adipates, azelates, sebacates and phthalates.

7. The flame-retardant hydraulic oil of claim 1, wherein the anti-load and anti-abrasive additive comprises an amine salt compound of phosphate ester represented by Formula 4: where R represents hydrogen or a C1 to C10 alkyl or aryl hydrocarbon compound, X represents hydrogen or C1 to C4 hydrocarbon, and n is an integer from 1 to 10.
